

# UNITED STATES PATENT OFFICE.

JULIUS RACZ, OF DETROIT, MICHIGAN, ASSIGNOR TO PERFECTION SHINGLE & ROOFING COMPANY, OF DETROIT, MICHIGAN, A CORPORATION OF MICHIGAN.

## ROOFING COMPOUND.

1,087,400.

Specification of Letters Patent. Patented Feb. 17, 1914.

No Drawing.

Application filed January 15, 1912. Serial No. 671,221.

*To all whom it may concern:*

Be it known that I, JULIUS RACZ, a subject of the Emperor of Austria-Hungary, residing at Detroit, in the county of Wayne 5 and State of Michigan, have invented certain new and useful Improvements in Roofing Compounds, of which the following is a specification.

The present invention consists of a special 10 material or compound composed of certain constituents or ingredients combined in a novel and advantageous manner.

The material derived by compounding in accordance with this invention has been 15 found most useful for roofing purposes in building because of its fire and weather proof qualities, and a peculiar elasticity, which it obtains in the process of manufacturing. This elasticity of the compound 20 or material aforesaid is quite necessary in order to reduce to a minimum any tendency of the same to become brittle, fragile, and readily chipped away or broken by the wear and tear of handling and commercial use.

In order that those skilled in the art to which this invention relates may produce the same, the preferred proportions and ingredients of the compound are as follows: 25 35 parts Japan drier, 35 parts iron filings, 30 15 parts ashes, 8 parts charcoal, 10 parts to 20 parts sand.

The above substances and materials are mixed in substantially the proportions specified and are then permitted to ripen or develop until they are thoroughly and effectively combined. The mixture is then rolled out upon or otherwise applied to a layer or strip of paper or equivalent material and 35 after going through a drying process the constituents of the compound not only become united but form with the paper a practically homogeneous product by virtue of

the fact that the compound closely adheres to the paper and penetrates the same. This product may be employed in many different 45 ways in building operations, as well as for other purposes, and is light, elastic, non-frangible, unaffected by changes in weather conditions, is waterproof and fireproof and cheap as a commercial article. In fact it 50 has been found that the elasticity of the product increases with age.

The Japan drier serves to firmly unite the iron, ashes, and sand, the mixture of these 55 four ingredients producing an elastic and flexible compound; the iron affords a requisite hardness, the sand affords a body, and the charcoal accelerates the drying of the materials in the manufacturing process.

For making shingles this product aforesaid has been found exceptionally advantageous as compared with slate, and its fire 60 proof qualities render it highly desirable to use in connection with fire-proof building construction.

The paper carrier when combined with the substances and materials recited is so united therewith by the chemical action of the elements of the product that said paper 65 cannot be separated from the ingredients 70 mentioned.

Having thus described the invention what is claimed as new is:

A roofing compound consisting of Japan 75 drier 35 parts, iron filings 35 parts, ashes 15 parts, charcoal 8 parts, and sand 10 to 20 parts, said compound being capable of adhering to and penetrating paper.

In testimony whereof I affix my signature in presence of two witnesses.

JULIUS RACZ.

Witnesses:

H. R. WUNDERLICH,  
FRANK HORALEKE.